# EUROPEAN PATENT SPECIFICATION

(11) **EP 0 280 115 B1**
(45) Date of publication and mention of the grant of the patent: **13.01.1993**
(21) Application number: 88101967.3
(22) Date of filing: 10.02.1988
(51) Int. Cl.: D21H 17/72, D21H 17/11, D21H 17/00

(54) **Oil proof composition for paper**
Ölabstossende Zusammensetzung für Papier
Composition répulsive de l'huile pour papier

(30) Priority: 12.02.1987 JP 30003/87
(43) Date of publication of application: 31.08.1988
(73) Proprietor: DAIKIN INDUSTRIES, LIMITED, Osaka-shi, Osaka-fu 530 (JP)
(72) Inventor: Aoyama, Hirokazu, Takatsuki-shi Osaka-fu (JP); Amimoto, Yoshio, Takatsuki-shi Osaka-fu (JP)
(74) Representative: Hansen, Bernd, Dr. Dipl.-Chem.

(56) References cited:
- GB-A- 2 117 021
- US-A- 3 953 283
- ABSTRACTS BULLETIN OF THE INSTITUTE OF PAPER CHEMISTRY, vol. 52, no. 11, May 1982, page 1347, abstract no. 12816, Appleton, Wisconsin, US

## Description

### BACKGROUND OF THE INVENTION

### Field of the Invention

The present invention relates to an oil proof composition for paper. More particularly, it relates to a composition for imparting oil resistance to paper which comprises a salt of fluorophosphate or a salt of fluorophosphonate and at least one anionic surfactant.

### Description of the Prior Arts

As oil proof agents for paper, namely sizing agents added to the paper in order to render the sheet more resistant to penetration of oils, salts of fluoroalkyl phosphate or salts of N-alkyl fluoroalkanesulfonamidoalkyl phosphate are known. Such conventional oil proof agents are applied to paper either by internal addition (internal sizing) which comprises dissolving or dispersing the agent in a pulp suspension or slurry for paper making, or by external addition (surface sizing) which comprises dipping a sheet of paper in an aqueous solution or dispersion of the agent or brushing over the sheet with the solution or dispersion to coat the surface of paper with the agent. In either of these additions, when water has too high hardness, the oil proof agent can be dissolved in a small amount of hard water. However, when the agent is added to a large amount of hard water or the aqueous solution of the agent is diluted with a large amount of hard water, the salt of fluoroalkyl phosphate or the salt of N-alkyl fluoroalkanesulfonamidoalkyl phosphate is precipitated, which results in decrease of sizing effect or deterioration of oil resistance of processed paper. When other finishing agents such as aluminum sulfate is used, the same drawback arises as when hard water is used.

A salt of fluoroalkenyloxyaralkyl phosphonate may be used as an oil proof agent for paper. But, it has the same drawback as the salt of fluoroalkyl phosphat when it is used in hard water.

US-A-3953283 discloses a process for preparing oil resistant paperboard from cellulosic pulp. The process comprises forming a suspension of cellulosic pulp, and then adding to this a mixture of (1) a cationically active material, (2) a water soluble salt of a saturated fatty acid, and (3) a water soluble bis-perfluorosulfonamino alkyl phosphate of specific formula.

Abstracts Bulletin of the Institute of Paper Chemistry, Vol. 52, No. 11, May 1982, page 1347, Abstract No. 12816 discloses the use of a dispersed phosphate containing perfluoro-alkyl or alkenyl groups for imparting oil-resistance to paper.

### SUMMARY OF THE INVENTION

An object of the present invention is to provide an oil proof composition for paper which is not precipitated in hard water and can impart good oil resistance to paper.

According to the present invention, this and other objects are achieved by an oil proof composition for paper which comprises at least one salt selected from the group consisting of fluoroalkyl phosphate salts, N-alkyl fluoroalkanesulfonamidoalkyl phosphate salts and fluoroalkenyloxyaralkyl phosphonate salts and at least one anionic surfactant.

### DETAILED DESCRIPTION OF THE INVENTION

The salt of fluoroalkyl phosphate may be a salt of the formula:

(R_{f}¹-A¹-O)ₘPO(OX¹)₃₋ₘ (I)

wherein R_{f}¹ is each a C₅-C₂₁ perfluoroalkyl or ω-hydroperfluoroalkyl group, A¹ is each a C₁-C₁₀ alkylene group, X¹ is an alkali metal or an ammonium group which may be substituted by a C₁-C₁₀ alkyl or hydroxyalkyl group, and m is 1 or 2. Preferred salts (I) are
(C₈F₁₇CH₂CH₂O)₂PO-ONH₂(C₂H₄OH)₂
C₈F₁₇CH₂CH₂OPO[ONH₂(C₂H₄OH)₂]₂
(C₆F₁₃CH₂CH₂O)₂PO-ONH₂(C₂H₄OH)₂
(C₁₀F₂₁CH₂CH₂O)₂PO-ONH₂(C₂H₄OH)₂
(C₁₂F₂₅CH₂CH₂O)₂PO-ONH₂(C₂H₄OH)₂
(C₁₄F₂₉CH₂CH₂O)₂PO-ONH₂(C₂H₄OH)₂
(C₈F₁₇CH₂CH₂O)₂PO-ONH₄
C₈F₁₇CH₂CH₂OPO(ONH₄)₂
(C₈F₁₇CH₂CH₂O)₂PO-ONH(C₂H₄OH)₃
(HC₆F₁₂CH₂O)₂PO-ONH₂(C₂H₄OH)₂
HC₆F₁₂CH₂CH₂OPO[ONH₂(C₂H₄OH)₂]₂
The salt of N-alkyl fluoroalkanesulfonamidoalkyl phosphate may be a salt of the formula:
wherein R_{f}² is each a C₅-C₂₁ perfluoroalkyl group, A² is each a C₁-C₁₀ alkyl group, A³ is each a C₁-C₁₀ alkylene group, X² is an alkali metal or or an ammonium group which may be substituted by a C₁-C₁₀ alkyl or hydroxyalkyl group, and n is 1 or 2. Preferred salts (II) are
[C₈F₁₇SO₂N(C₂H₅)CH₂CH₂O]₂PO-ONH₄
C₈F₁₇SO₂N(C₂H₅)CH₂CH₂OPO(ONH₄)₂
[C₆F₁₃SO₂N(C₂H₅)CH₂CH₂O]₂PO-ONH₄
[C₁₀F₂₁SO₂N(C₂H₅)CH₂CH₂O]₂PO-ONH₄
[C₁₂F₂₅SO₂N(C₂H₅)CH₂CH₂O]₂PO-ONH₄
[C₁₄F₂₉SO₂N(C₂H₅)CH₂CH₂O]₂PO-ONH₄
[C₈F₁₇SO₂N(C₂H₅)CH₂CH₂O]₂PO-ONH₂(CH₂CH₂OH)₂
C₈F₁₇SO₂N(C₂H₅)CH₂CH₂OPO[ONH₂(CH₂CH₂OH)₂]₂
[C₈F₁₇SO₂N(C₂H₅)CH₂CH₂O]₂PO-ONH₂(CH₂CH₂OH)₃
The salt of fluoroalkenyloxyaralkyl phosphonate may be a salt of the formula:

(R_{f}³O)ₚAr(CH₂)_{q}PO(OX³)₂ (III)

wherein R_{f}³ is each a C₆-C₁₂ perfluoroalkenyl group, p is 1, 2 or 3 and Ar is an aromatic group which may have a substituent (e.g. phenyl, naphthyl, or alkyl-, acyl-, alkoxy- or halogen-substituted phenyl or naphthyl), q is 1 or 2 and X³ is an alkali metal or an ammonium group which may be substituted by a C₁-C₁₀ alkyl or hydroxyalkyl group. Preferred salts (III) are
C₆F₁₁O-C₆H₄-CH₂PO(ONa)₂
C₉F₁₇O-C₆H₄-CH₂PO(ONH₄)₂
C₉F₁₇O-C₆H₄-CH₂PO[ONH₂(C₂H₄OH)₂]₂
C₉F₁₇O-C₆H₄-CH₂CH₂PO(ONa)₂
The above salt of phosphate or phosphonate may be prepared by neutralizing at least one partial ester selected from the group consisting of fluoroalkyl partial esters of phosphoric acid, N-alkyl fluoroalkanasulfoneamidoalkyl partial esters of phosphoric acid and fluoroalkenyloxyaralkyl partial esters of phosphonic acid with a base (e.g. hydroxides of alkali metals, amines, etc.) according to a conventional method.

The anionic surfactant is preferably a hydrocarbon type anionic surfactant. Examples of the anionic surfactant are C₅-C₁₅ alkylbenzenesulfonic acids, C₅-C₁₅ alkylbenzenesulfonate salts, di-C₅-C₁₅ alkyl sulfosuccinate salts, C₉-C₂₁ alkyl sulfate salts, C₁₀-C₂₀ alkylsulfonate salts, C₃-C₁₅ alkylnaphthalenesulfonate salts, mono- or di-C₉-C₂₁ alkyl phosphate salts, salts of C₉-C₂₅ fatty acids and the like. The salt may be a sodium, potassium, ammonium, mono-, di- or tri-C₁-C₅ alkyl or hydroxyalkylammonium salt.

The amount of anionic surfactant is from 1 to 15 % by weight based on the weight of phosphate or phosphonate which is converted to the weight of corresponding partial ester.

The oil proof composition of the present invention may be used together with other processing agents such as a bonding agent such as Sumilets resin FC-50L and Sumilets resin 675 (both available from Sumitomo Chemical Co., Ltd.). The amount of bonding agent is from 0.5 to 3 times by weight based on the weight of oil proof composition (the weight of the salt of fluorophosphate and/or fluorophosphonate being converted to a weight of corresponding partial ester).

The oil resistant imparting composition is easily prepared by mixing the salt of phosphate or phosphonate and the anionic surfactant.

Oil resistant imparting composition of the present invention is not precipitated when diluted with comparatively hard water or water containing aluminum sulfate, or when stirred vigorously. Even when the oil proof composition is added to paper by the internal addition, paper has good properties such as sizing degree in addition to oil resistance.

The present invention will be illustrated by following examples, in which "%" is by weight unless otherwise indicated.

### Example 1

### Preparation Example

In a 4 liter round flask equipped with a stirrer, CF₃CF₂(CF₂CF₂)ₙCH₂CH₂OH (n=2, 1 % by mole; n=3, 55 % by mole; n=4, 26 % by mole; n=5, 12 % by mole; n=6, 5 % by mole; n=7, 1 % by mole) (300 g) and 85 % phosphoric acid (6.4 g) were charged, and phosphorus oxychloride (33.8 g) was added at a temperature of 80 to 85°C with stirring over 30 minutes. After purging hydrogen chloride gas under reduced pressure, water (28 g) was added and stirred at a temperature of 95 to 100°C for 1 hour. Thereafter, the mixture was cooled to 85°C and isopropanol (66 g) was added to prepare a phosphate ester stock solution having the following composition:

| | |
|---|---|
| CF₃CF₂(CF₂CF₂)ₙCH₂CH₂OH | 0.75 % |
| CF₃CF₂(CF₂CF₂)ₙCH₂CH₂OPO(OH)₂ | 8.45 % |
| [CF₃CF₂(CF₂CF₂)ₙCH₂CH₂O]₂POOH | 53.24 % |
| [CF₃CF₂(CF₂CF₂)ₙCH₂CH₂O]₃PO | 15.89 % |
| Water | 3.82 % |
| Isopropanol | 17.85 % |

### Example 1

In a 4 liter round flask equipped with a stirrer, the phosphate ester stock solution prepared in Preparation Example (400 g) was charged followed by addition of diethanolamine (110 g) at a temperature of 70 to 75°C. Then, sodium salt of dodecyl benzenesulfonate (16 g, 6.5 % per weight of the phosphate salt) and warm water (50 g) were added followed by addition of warm water (1,500 g) to give an emulsion of oil proof agent (pH 10) having the following composition:

### Example 2

In the same manner as in Example 1 but using 5.4 g (2.2 % per weight of the phosphate) of sodium salt of dodecyl benzenesulfonate, an emulsion of oil proof agent (pH 10) was prepared.

### Example 3

To the emulsion of oil proof agent prepared in Example 1, hydrochloric acid was added to give an emulsion of oil proof agent having pH of 7.

### Example 4

In the same manner as in Example 1 but using 16 g of sodium salt of dioctyl sulfosuccinate in place of sodium salt of dodecyl benzenesulfonate, an emulsion of oil proof agent (pH 10) was prepared.

### Example 5

In the same manner as in Example 1 but using 28 % ammonia water (110 g) in place of diethanolamine, an emulsion of oil proof agent (pH 10) was prepared.

### Example 6

In the same manner as in Example 5 but using 16 g of sodium dioctylsulfosuccinate in place of sodium salt of dodecyl benzenesulfonate, an emulsion of oil proof agent (pH 10) was prepared.

### Example 7

In the same manner as in Example 6 but using 11.2 g of sodium dioctylsulfosuccinate (4.5 % per weight of the phosphate), an emulsion of oil proof agent (pH 10) was prepared.

### Examples 8 and 9

To the emulsion of oil proof agent obtained in Example 6, hydrochloric acid was added to give an emulsion of oil proof agent having pH of 9 (Example 8) or pH of 7 (Example 9).

### Comparative Example 1

In the same manner as in Example 1 but using no surfactant, an emulsion of oil proof agent was prepared.

### Comparative Example 2

In the same manner as in Example 5 but using no surfactant, an emulsion of oil proof agent was prepared.

The compositions and pH values of the oil proof compositions prepared in Examples and Comparative Examples are summarized in Table 1.

### Experiment 1

Dilution stability of the emulsion of oil proof agent prepared in Example 2 or Comparative Example 1 was examined.

The emulsion was diluted with water having various hardness to adjust the concentration of the oil proof agent to 1 %. Then, one portion of the diluted emulsion was stirred at 3,000 ppm for 3 minutes while another portion was not stirred. Then, both were kept standing for one day and a precipitated amount per 10 ml was measured. The results are shown in Table 2.

**Table 2**

| | Hardness of water (CaCO₃) | Precipitated amount (ml) | |
|---|---|---|---|
| | | Stirring | No stirring |
| Example 2 | 0 | 0 | 0.01 |
| | 100 | 0.01 | 0.10 |
| | 200 | 0.01 | 0.12 |
| | 300 | 0.01 | 0.20 |
| Comparative Example 1 | 0 | 0 | 0.50 |
| | 100 | 0.02 | 1.92 |
| | 200 | 0.03 | 2.11 |

### Experiment 2

Stability against aluminum sulfate of the same emulsions of oil proof agents as used in Experiment 1 was examined.

To 100 ml of the emulsion containing 0.5 % of the oil proof agent, 0.2 ml or 0.5 ml of a 1 % aqueous solution of aluminum sulfate was dropwise added and kept standing at room temperature for 1 hour. Just after the addition of aluminum sulfate and after kept standing for 1 hour, a precipitation state was observed and evaluated according to the following criteria:
- O:: No precipitate
- △:: Few precipitates
- X:: A few precipitates
- XX:: Many precipitates
The results are shown in Table 3.

**Table 3**

| | 0.2 ml addition | | 0.5 ml addition | |
|---|---|---|---|---|
| | Just after addition | After 1 hour | Just after addition | After 1 hour |
| Example 2 | O | O | △ | △ |
| Comparative Example 1 | △ | X | X | XX |

### Experiment 3

Mechanical stability of the emulsion of oil proof agent was evaluated.

Each of the emulsions of oil proof agents prepared in Examples 1-9 and Comparative Examples 1 and 2 was stirred at 3,000 rpm for 3 minutes and condition of the emulsion was observed and evaluated according to the following criteria:
- OO:: No precipitate
- O:: Few precipitates
- △:: A few precipitates
- X:: Many precipitates
The results are shown in Table 4.

**Table 4**

| Example No. | Mechanical Stability | Sumilets resin FC-50L | | Sumilets resin 675 | |
|---|---|---|---|---|---|
| | | Oil resistance | Sizing degree | Oil resistance | Sizing degree |
| 1 | O | 12 | 4.1 | 12 | 26.4 |
| 2 | O | 12.5 | 4.9 | 12.5 | 25.8 |
| 3 | O | 12 | 3.6 | 11.5 | 20.9 |
| 4 | △ | 13 | 3.9 | 11.5 | 18.4 |
| 5 | O | 13⁺ | 5.1 | 11 | 19.2 |
| 6 | OO | 13⁺ | 3.6 | 11⁺ | 19.1 |
| 7 | OO | 14 | 3.3 | 11⁺ | 20.2 |
| 8 | OO | 14 | 4.4 | 11.5 | 21.4 |
| 9 | OO | 14 | 3.1 | 10 | 12.9 |
| Com. 1 | X | 12 | 2.3 | 11.5 | 17.9 |
| Com. 2 | X | 13 | 3.0 | 11.5 | 18.6 |

### Experiment 4

A sizing effect of each of the emulsions of oil proof agents prepared in Examples 1-9 and Comparative Examples 1 and 2 was evaluated. By using, as a bonding agent, Sumilets resin FC-50L (0.2 % per weight of pulp) or Sumilets 675 (0.3 % per weight of pulp), the oil proof composition (0.35 % of solid materials per weight of pulp) was added to paper by the internal addition method.

The sizing degree was measured as follows:
From a sheet of paper containing the oil proof composition, a square piece of paper (50 mm x 50 mm) was cut out and its peripheral parts were folded upwardly along lines about 1 cm inside from and in parallel with the four edge lines to make a small box. As soon as the box was placed on a surface of a 2 % aqueous solution of ammonium rhodanate in a petri dish kept at 20±1°C, a drop of a 1 % aqueous solution of ferric chloride kept at the same temperature was added in the box. Then, a period of time till three red spots appeared on the bottom of the paper box was measured.
The sizing effect was expressed in terms of such period of time. The results are shown in Table 4.

### Experiment 5

Oil resistance of the paper as prepared in Experiment 4 was evaluated as follows:
Castor oil (chemically pure (c.p.) grade), toluene (c.p. grade) and heptane (c.p. grade) were mixed in a ratio shown in Table 5 to prepare mixed solvent Nos. 1 to 16. Then, each mixed solvent was dropped on a sheet of paper placed on a clean flat surface from a height of about 2.5 cm above the sheet of paper. After 15 seconds from the completion of dropping of the mixed solvent, conditions of the paper sheet where the mixed solvent was dropped were observed. When any black spot was formed, the oil resistance was evaluated as "unacceptable" irrespective of the area of the spot, while no spot was formed, the oil resistance was evaluated as "acceptable". The oil resistance was expressed in terms of the maximum number of mixed solvent for which the oil resistance was acceptable. The larger the number of mixed solvent, the better the oil resistance of paper. The results are also shown in Table 4 above.

**Table 5**

| Mixed solvent No. | Castor oil (ml) | Toluene (ml) | Heptane (ml) |
|---|---|---|---|
| 1 | 200 | 0 | 0 |
| 2 | 180 | 10 | 10 |
| 3 | 160 | 20 | 20 |
| 4 | 140 | 30 | 30 |
| 5 | 120 | 40 | 40 |
| 6 | 100 | 50 | 50 |
| 7 | 80 | 60 | 60 |
| 8 | 60 | 70 | 70 |
| 9 | 40 | 80 | 80 |
| 10 | 20 | 90 | 90 |
| 11 | 0 | 100 | 100 |
| 12 | 0 | 90 | 110 |
| 13 | 0 | 70 | 130 |
| 14 | 0 | 50 | 150 |
| 15 | 0 | 30 | 170 |
| 16 | 0 | 0 | 200 |

### Example 10

In a 4 liter round flask equipped with a stirrer, the phosphate ester stock solution prepared in Preparation Example (400 g) was charged followed by addition of diethanolamine (110 g) at a temperature of 70 to 75°C. Then, sodium salt of dodecyl benzenesulfonate (7.4 g, 3.0 % per weight of the phosphate salt) and warm water (50 g) were added followed by addition of warm water (1,500 g) to give an emulsion of oil proof agent (pH 10) having the following composition:

### Comparative Example 3

In the same manner as in Example 10 but using Nonion HS-220 (a nonionic surfactant,
in which an average of n is 20 manufactured by Nippon Oil and Fat Co., Ltd.) (7.4 g) in plase of the sodium salt of dodecyl benzenesulfonate, an emulsion of oil proof agent was prepared.

### Experiment 6

Stability against dilution with hard water of the emulsion of oil proof agent prepared in Example 10 or Comparative Example 3 was examined.

The emulsion was diluted with water containing 50 ppm of Ca²⁺ to adjust the concentration of the oil proof agent to 1 % or with water containing 75 ppm of Ca²⁺ to adjust the concentration of the oil proof agent to 0.2 %. Then, each diluted emulsion was stirred at 3,000 ppm for 3 minutes. The conditon of the emulsion was observed and evaluated according to the same criteria as used in Experiment 3. The results are shown in Table 5.

### Experiment 7

A sizing effect of each of the emulsions of oil proof agents prepared in Experiment 6 was evaluated.

To a 60 g/l pulp suspension, as a bonding agent, Sumilets resin FR-2P (0.3 % per weight of pulp) and the oil proof composition (0.25, 0.30 or 0.35 % of solid materials per weight of pulp) was added to paper by the internal addition method. The average weight of paper was 60 g/m².

The sizing degree was measured in the same manner as in Experiment 4. The results are shown in Table 5.

### Experiment 8

Oil resistance of the paper prepared in Experiment 7 was evaluated in the same manner as in Experiment 5.

The results are shown in Table 5.

**Table 5**

| | Dilution stability (CaCO₃) | | Sizing degree | | | Oil resistance | | |
|---|---|---|---|---|---|---|---|---|
| Concentration of phosphate salt (%) | 1 | 0.2 | 0.25 | 0.30 | 0.35 | 0.25 | 0.30 | 0.35 |
| | Ca²⁺ 50 ppm | Ca²⁺ 75 ppm | | | | | | |
| Example 10 | O | △ | 3 | 6 | 8 | 8 | 12 | 12 |
| Comparative Example 3 | △ | X | 2 | 2 | 5 | 8 | 10 | 10 |

## Claims

1. An oil proof composition for paper which comprises at least one anionic surfactant and a fluorine-containing compound, characterised in that the fluorine-containing compound is at least one of a fluoroalkyl phosphate salt, an N-alkyl fluoroalkanesulfonamidoalkyl phosphate salt and a fluoroalkenyloxyaralkyl phosphonate salt.

2. The oil proof composition according to claim 1, wherein the salt is a salt of fluoroalkyl phosphate of the formula:
(R_{f}¹-A¹-O)ₘPO(OX¹)₃₋ₘ
wherein R_{f}¹ is each a C₅-C₂₁ perfluoroalkyl or ω-hydroperfluoroalkyl group, A¹ is each a C₁-C₁₀ alkylene group, X¹ is an alkali metal or an ammonium group which may be substituted by a C₁-C₁₀ alkyl or hydroxyalkyl group, and m is 1 or 2.

3. The oil proof composition according to claim 2, wherein the salt of fluoroalkylphosphate is a salt of the formula:
(C₈F₁₇CH₂CH₂O)₂PO-ONH₂(C₂H₄OH)₂
C₈F₁₇CH₂CH₂OPO[ONH₂(C₂H₄OH)₂]₂
(C₆F₁₃CH₂CH₂O)₂PO-ONH₂(C₂H₄OH)₂
(C₁₀F₂₁CH₂CH₂O)₂PO-ONH₂(C₂H₄OH)₂
(C₁₂F₂₅CH₂CH₂O)₂PO-ONH₂(C₂H₄OH)₂
(C₁₄F₂₉CH₂CH₂O)₂PO-ONH₂(C₂H₄OH)₂
(C₈F₁₇CH₂CH₂O)₂PO-ONH₄
C₈F₁₇CH₂CH₂OPO(ONH₄)₂
(C₈F₁₇CH₂CH₂O)₂PO-ONH(C₂H₄OH)₃
(HC₆F₁₂CH₂O)₂PO-ONH₂(C₂H₄OH)₂ or
HC₆F₁₂CH₂CH₂OPO[ONH₂(C₂H₄OH)₂]₂.

4. The oil proof composition according to claim 1, wherein the salt is a salt of N-alkyl fluoroalkanesulfonamidoalkyl phosphate of the formula: wherein R_{f}² is each a C₅-C₂₁ perfluoroalkyl group, A² is each a C₁-C₁₀ alkyl group, A³ is each a C₁-C₁₀ alkylene group, X² is an alkali metal or or an ammonium group which may be substituted by a C₁-C₁₀ alkyl or hydroxyalkyl group, and n is 1 or 2.

5. The oil proof composition according to claim 4, wherein the salt of N-alkyl fluoroalkanesulfonamidoalkyl phosphate is a salt of the formula:
[C₈F₁₇SO₂N(C₂H₅)CH₂CH₂O]₂PO-ONH₄
C₈F₁₇SO₂N(C₂H₅)CH₂CH₂OPO(ONH₄)₂
[C₆F₁₃SO₂N(C₂H₅)CH₂CH₂O]₂PO-ONH₄
[C₁₀F₂₁SO₂N(C₂H₅)CH₂CH₂O]₂PO-ONH₄
[C₁₂F₂₅SO₂N(C₂H₅)CH₂CH₂O]₂PO-ONH₄
[C₁₄F₂₉SO₂N(C₂H₅)CH₂CH₂O]₂PO-ONH₄
[C₈F₁₇SO₂N(C₂H₅)CH₂CH₂O]₂PO-ONH₂(CH₂CH₂OH)₂
C₈F₁₇SO₂N(C₂H₅)CH₂CH₂OPO[ONH₂(CH₂CH₂OH)₂]₂ or
[C₈F₁₇SO₂N(C₂H₅)CH₂CH₂O]₂PO-ONH₂(CH₂CH₂OH)₃.

6. The oil proof composition according to claim 1, wherein the salt is a salt of fluoroalkenyloxyaralkyl phosphonate of the formula:
(R_{f}³O)ₚAr(CH₂)_{q}PO(OX³)₂
wherein R_{f}³ is each a C₆-C₁₂ perfluoroalkenyl group, p is 1, 2 or 3 and Ar is an aromatic group which may have a substituent (e.g. phenyl, naphthyl, or alkyl-, acyl-, alkoxy- or halogen-substituted phenyl or naphthyl), q is 1 or 2 and X³ is an alkali metal or an ammonium group which may be substituted by a C₁-C₁₀ alkyl or hydroxyalkyl group.

7. The oil proof composition according to claim 1, wherein the salt of fluoroalkeneyloxyaralkyl phosphate is a salt of the formula:
C₆F₁₁O-C₆H₄-CH₂PO(ONa)₂
C₉F₁₇O-C₆H₄-CH₂PO(ONH₄)₂
C₉F₁₇O-C₆H₄-CH₂PO[ONH₂(C₂H₄OH)₂]₂ or
C₉F₁₇O-C₆H₄-CH₂CH₂PO(ONa)₂.

## Patentansprüche

1. Ölbeständige Zusammensetzung für Papier, welche mindestens ein anionisches Tensid und eine fluorhaltige Verbindung umfaßt, dadurch **gekennzeichnet,** daß die fluorhaltige Verbindung mindestens ein Fluoroalkylphosphatsalz, N-Alkylfluoroalkansulfonamidoalkyl-phosphatsalz und/oder Fluoroalkenyloxyaralkyl-phosphonatsalz ist.

2. Ölbeständige Zusammensetzung gemäß Anspruch 1, worin das Salz ein Fluoroalkylphosphatsalz der Formel
(R_{f}¹-A¹-O)ₘPO(OX¹)₃₋ₘ
ist, worin R_{f}¹ jeweils eine C₅-C₂₁-Perfluoroalkyl- oder ω-Hydroperfluoroalkyl-Gruppe ist, A¹ jeweils eine C₁-C₁₀-Alkylen-Gruppe ist, X¹ ein Alkalimetall oder eine Ammonium-Gruppe ist, welche durch eine C₁-C₁₀-Alkyl- oder -Hydroxyalkyl-Gruppe substituiert sein kann, und m 1 oder 2 ist.

3. Ölbeständige Zusammensetzung gemäß Anspruch 2, worin das Fluoroalkylphosphatsalz ein Salz der Formel ist:
(C₈F₁₇CH₂CH₂O)₂PO-ONH₂(C₂H₄OH)₂
C₈F₁₇CH₂CH₂OPO[ONH₂(C₂H₄OH)₂]₂
(C₆F₁₃CH₂CH₂O)₂PO-ONH₂(C₂H₄OH)₂
(C₁₀F₂₁CH₂CH₂O)₂PO-ONH₂(C₂H₄OH)₂
(C₁₂F₂₅CH₂CH₂O)₂PO-ONH₂(C₂H₄OH)₂
(C₁₄F₂₉CH₂CH₂O)₂PO-ONH₂(C₂H₄OH)₂
(C₈F₁₇CH₂CH₂O)₂PO-ONH₄
C₈F₁₇CH₂CH₂OPO(ONH₄)₂
(C₈F₁₇CH₂CH₂O)₂PO-ONH(C₂H₄OH)₃
(HC₆F₁₂CH₂O)₂PO-ONH₂(C₂H₄OH)₂
HC₆F₁₂CH₂CH₂OPO[ONH₂(C₂H₄OH)₂]₂

4. Ölbeständige Zusammensetzung gemäß Anspruch 1, worin das Salz ein N-Alkylfluoroalkansulfonamidoalkylphosphatsalz der Formel ist, worin R_{f}² jeweils eine C₅-C₂₁-Perfluoroalkyl-Gruppe ist, A² jeweils eine C₁-C₁₀-Alkyl-Gruppe ist, A³ jeweils eine C₁-C₁₀-Alkylen-Gruppe ist, X² ein Alkalimetall oder eine Ammonium-Gruppe ist, welche durch eine C₁-C₁₀-Alkyl- oder Hydroxyalkyl-Gruppe substituiert sein kann, und n 1 oder 2 ist.

5. Ölbeständige Zusammensetzung gemäß Anspruch 4, worin das N-Alkylfluoroalkansulfonamidoalkyl-phosphatsalz ein Salz der Formel ist:
[C₈F₁₇SO₂N(C₂H₅)CH₂CH₂O]₂PO-ONH₄
C₈F₁₇SO₂N(C₂H₅)CH₂CH₂OPO(ONH₄)₂
[C₆F₁₃SO₂N(C₂H₅)CH₂CH₂O]₂PO-ONH₄
[C₁₀F₂₁SO₂N(C₂H₅)CH₂CH₂O]₂PO-ONH₄
[C₁₂F₂₅SO₂N(C₂H₅)CH₂CH₂O]₂PO-ONH₄
[C₁₄F₂₉SO₂N(C₂H₅)CH₂CH₂O]₂PO-ONH₄
[C₈F₁₇SO₂N(C₂H₅)CH₂CH₂O]₂PO-ONH₂(CH₂CH₂OH)₂
C₈F₁₇SO₂N(C₂H₅)CH₂CH₂OPO[ONH₂(CH₂CH₂OH)₂]₂ oder
[C₈F₁₇SO₂N(C₂H₅)CH₂CH₂O]₂PO-ONH₂(CH₂CH₂OH)₃.

6. Ölbeständige Zusammensetzung gemäß Anspruch 1, worin das Salz ein Fluoroalkenyloaralkyl-phosphonatsalz der Formel ist:
(R_{f}³O)ₚAr(CH₂)_{q}PO(OX³)₂
worin R_{f}³ jeweils eine C₆-C₁₂-Perfluoroalkenyl-Gruppe ist, p 1, 2 oder 3 ist, und Ar eine aromatische Gruppe ist, welche einen Substituenten (z.B. Phenyl, Naphthyl oder alkyl-, acyl-, alkoxy- oder halogensubstituiertes Phenyl oder Naphthyl) haben kann, q 1 oder 2 ist und X³ ein Alkalimetall oder eine Ammonium-Gruppe ist, welche durch eine C₁-C₁₀-Alkyl- oder -Hydroxyalkyl-Gruppe substituiert sein kann.

7. Ölbeständige Zusammensetzung gemäß Anspruch 1, worin das Fluoroalkenyloxyaralkyl-phosphonatsalz ein Salz der Formel ist:
C₆F₁₁O-C₆H₄-CH₂PO(ONa)₂
C₉F₁₇O-C₆H₄-CH₂PO(ONH₄)₂
C₉F₁₇O-C₆H₄-CH₂PO[ONH₂(C₂H₄OH)₂]₂
C₉F₁₇O-C₆H₄-CH₂CH₂PO(ONa)₂

## Revendications

1. Une composition d'imperméabilisation à l'huile pour papier qui comprend au moins un agent surfactant anionique et un composé contenant du fluor, caractérisée en ce que le composé contenant du fluor est au moins l'un des suivants : un sel de phosphate de fluoroalkyle, un sel de phosphate de N-alkyle fluoroalcanesulfonamidoalkyle, et un sel de phosphonate de fluoroalcényloxyaralkyle.

2. La composition d'imperméabilisation à l'huile selon la revendication 1, selon laquelle le sel est un sel de phosphate de fluoroalkyle de formule :
(R_{f}¹-A¹-O)ₘPO(OX¹)₃₋ₘ (I)
dans laquelle R_{f}¹ désignent chacun un groupe C₅-C₂₁ perfluoroalkyle ou ω-hydroperfluoroalkyle, A¹ désignent chacun un groupe C₁-C₁₀ alkylène, X₁ est un métal alcalin ou un groupe ammonium qui peut être substitué par un groupe C₁-C₁₀ alkyle ou hydroxyalkyle, et m est égal à 1 ou 2.

3. La composition d'imperméabilisation à l'huile conformément à la revendication 2, selon laquelle le sel de phosphate de fluoroalkyle est un sel de formule :
(C₈F₁₇CH₂CH₂O)₂PO-ONH₂(C₂H₄OH)₂
C₈F₁₇CH₂CH₂OPO[ONH₂(C₂H₄OH)₂]₂
(C₆F₁₃CH₂CH₂O)₂PO-ONH₂(C₂H₄OH)₂
(C₁₀F₂₁CH₂CH₂O)₂PO-ONH₂(C₂H₄OH)₂
(C₁₂F₂₅CH₂CH₂O)₂PO-ONH₂(C₂H₄OH)₂
(C₁₄F₂₉CH₂CH₂O)₂PO-ONH₂(C₂H₄OH)₂
(C₈F₁₇CH₂CH₂O)₂PO-ONH₄
C₈F₁₇CH₂CH₂OPO(ONH₄)₂
(C₈F₁₇CH₂CH₂O)₂PO-ONH(C₂H₄OH)₃
(HC₆F₁₂CH₂O)₂PO-ONH₂(C₂H₄OH)₂ ou
HC₆F₁₂CH₂CH₂OPO[ONH₂(C₂H₄OH)₂]₂.

4. La composition d'imperméabilisation à l'huile conformément à la revendication 1, selon laquelle le sel est un sel de phosphate de N-alkyle fluoroalcanesulfonamidoalkyle de formule : dans laquelle R_{f}² désignent chacun un groupe C₅-C₂₁ perfluoroalkyle, A² désignent chacun un groupe C₁-C₁₀ alkyle, A³ désignent chacun un groupe C₁-C₁₀ alkylène, X² est un métal alcalin ou un groupe ammonium et peut être substitué par un groupe C₁-C₁₀ alkyle ou hydroxyalkyle, et n est égal à 1 ou 2.

5. La composition d'imperméabilisation à l'huile conformément à la revendication 4, selon laquelle le sel de phosphate de N-alkyle fluoroalcanesulfonamidoalkyle est un sel de formule :
[C₈F₁₇SO₂N(C₂H₅)CH₂CH₂O]₂PO-ONH₄
C₈F₁₇SO₂N(C₂H₅)CH₂CH₂OPO(ONH₄)₂
[C₆F₁₃SO₂N(C₂H₅)CH₂CH₂O]₂PO-ONH₄
(C₁₀F₂₁SO₂N(C₂H₅)CH₂CH₂O]₂PO-ONH₄
[C₁₂F₂₅SO₂N(C₂H₅)CH₂CH₂O]₂PO-ONH₄
[C₁₄F₂₉SO₂N(C₂H₅)CH₂CH₂O]₂PO-ONH₄
[C₈F₁₇SO₂N(C₂H₅)CH₂CH₂O]₂PO-ONH₂(CH₂CH₂OH)₂
C₈F₁₇SO₂N(C₂H₅)CH₂CH₂OPO[ONH₂(CH₂CH₂OH)₂]₂ ou
[C₈F₁₇SO₂N(C₂H₅)CH₂CH₂O]₂PO-ONH₂(CH₂CH₂OH)₃.

6. La composition d'imperméabilisation à l'huile selon la revendication 1, selon laquelle le sel est un sel de phosphonate de fluoroalcényloxyaralkyle de formule :
(R_{f}³O)ₚAr(CH₂)_{q}PO(OX³)₂
dans laquelle R_{f}³ désignent chacun un groupe C₆-C₁₂ perfluoroalcényle, p est égal à 1, 2 ou 3 et Ar est un groupe aromatique qui peut avoir un substituant (par exemple phényle, naphtyle, ou alkyl-, acyl-, alcoxy- ou halogéno-substitué phényle ou naphtyle), q est égal à 1 ou 2 et X³ est un métal alcalin ou un groupe ammonium qui peut être substitué par un groupe C₁-C₁₀ alkyle ou hydroxyalkyle.

7. La composition d'imperméabilisation à l'huile selon la revendication 1, selon laquelle le sel de phosphate de fluoroalcényloxyaralkyle est un sel de formule :
C₆F₁₁O-C₆H₄-CH₂PO(ONa)₂
C₉F₁₇O-C₆H₄-CH₂PO(ONH₄)₂
C₉F₁₇O-C₆H₄-CH₂PO[ONH₂(C₂H₄OH)₂]₂ ou
C₉F₁₇O-C₆H₄-CH₂CH₂PO(ONa)₂.
